

# UNITED STATES PATENT OFFICE.

WILHELM MENSING, OF FREIBERG, GERMANY.

## PROCESS FOR PRODUCING FERRO-LEATHER.

1,371,803.

Specification of Letters Patent. Patented Mar. 15, 1921.

No Drawing. Application filed January 23, 1917, Serial No. 144,099. Renewed January 27, 1921. Serial No. 440,530.

To all whom it may concern:

Be it known that I, WILHELM MENSING, a subject of the King of Prussia, German Emperor, residing at No. 5 Hainichenerstrasse, 5 Freiberg, Germany, in the Kingdom of Saxony, have invented new and useful Improvements in Processes for Producing Ferro-Leather; and I do hereby declare the following to be a full, clear, and exact description of the same.

According to the ferri-tanning processes heretofore known it is not possible to produce, without difficulty, a tough and perfectly durable leather, which is proof 10 against tearing and fracture, from ferri-salts obtained by oxidizing ferro-salts with chromic acid or nitric acid. This is due to the fact that the ferri-salt solutions have a very high dissociating capacity and therefore 15 incline to separate insoluble ferric compounds, which are formed particularly in the outer layers of the leather and thus produce a rough brittle grain.

Attempts have been made to overcome this 20 drawback of the ferro-tanning process by using ferri-salts, but in the presence of ferro-salts, which latter prevent the formation of basic ferri-salts. Although in this case 25 a rough brittle grain is avoided, still, owing to the mutable character of the ferro-salts, the quality of the leather is reduced by keeping, as is shown by the grain becoming brittle and by the leather being more easily torn.

Now it has been found that these 30 drawbacks are avoided, if, in preparing the ferric solutions and tanning liquor, as well as in the tanning process itself, care is taken, to prevent the hydrolytic splitting up of the ferri-salt, as far as possible, and to avoid 35 ferro-salts in the tanning liquor, or their formation in the leather.

In order to assure that no ferro-salts are contained in the tanning liquor, and to prevent 40 their subsequent formation in the leather, the tanning is carried out, according to the present invention, in the presence of an excess of oxidizing agents. When 45 making ferri-salt solutions from ferro-salts by oxidation with the assistance of chromic acid or nitric acid, or the like, such a quantity of this oxidizing agent is used that an 50 excess of the same remains in a non-reducible form.

It has been found that it is of special ad- 55 vantage to use oxidizing chlorid compounds

free from iron, such as sodium-chlorate, potassium-chlorate, barium-chlorate or chloric acid, instead of the usual oxidizing agents, such as chromic acid or nitric acid. The use of such chlorate compounds is cheaper than 60 chrome compounds and the process is simpler and more easily carried out than with nitric acid. Further a very durable leather is obtained which keeps well.

In order to obtain a perfect result, it is 65 necessary, as above set forth to prevent a hydrolytic splitting up of the ferri-salt. As high temperatures exercise a decomposing action on the ferri-salts it is advisable, in making the ferric solution, not to much exceed 70 35° C. and to then rapidly cool the solution down to the temperature of the room.

Because, further, dilute ferri-salt solutions split up relatively quickly into a basic salt and free acid, while, according as the 75 concentration increases, this splitting up does not occur so easily, it is advisable to use strong ferri-salt solutions for tanning, thus without the usual slow improvement of the tanning liquor.

If depilated skins ready for tanning are treated with concentrated solutions of a ferri-salt produced at a moderate temperature, which ferri-salt is perfectly free from 80 ferro-salt and contains a slight excess of an oxidizing agent, so that any ferro-salts which may happen to be present are oxidized, then leather of good marketable quality is obtained, which, according to experiments, after being kept for six years have 85 a good a quality as when first made.

By observing the directions and by suitable carrying out the process hard or soft flexible leather can be made, if the acid combined with the ferric oxid, beginning 90 with the most difficultly soluble basic salt, is increased until a weakly acid salt is obtained.

When using slightly acid or neutral ferri-salts the depilated skins from which the 100 lime has been separated are subjected to a preliminary treatment with slightly alkaline salts, such as borax, or they are firstly tanned with aluminium or chromic oxid salts rendered basic, so that any free acid 105 present may be combined.

### Example.

A ferri-salt solution of about 10%  $Fe_2O_3$  is produced either by dissolving in water 110

some ferri-salt for instance ferric sulfate or by oxidation of a ferro-salt solution, for instance ferrous sulfate by means of air or nitric acid.

5 Care should be taken when the solution is prepared that a temperature of 35° C. be not exceeded and a sufficient quantity of a non-volatile oxidation agent is added that there be always present in the 10% ferric 10 solution, 1% of that non-volatile oxidation agent in the free state. When the ferri-salt solution is prepared by oxidation of ferrous salts by means of chromic acid, nitric acid or chloric acid, so much of the oxidizing agent 15 must be added right away that there remains about 10% thereof in non-reduced state.

For tanning depilated skins which have been pickled and preliminarily tanned a suitable quantity of a  $\frac{2}{3}$ % solution of sodium 20 chlorid or sulfate of soda is produced, and a sufficient quantity of the ferric solution produced in the mean time is added to assure that the tanning liquor contains at least 1 to 2% ferric oxid ( $Fe_2O_3$ ), whereupon the 25 tannin process is commenced at once without further improvement. It is finished when a fresh cut shows a uniform tanning and no further reduction of the strength of the liquor can be ascertained.

30 By suitable finishing processes it is possible to give to the ferro-leather made in accordance with this invention further excellent properties.

The ferro-leather taken out of the tanning 35 liquor is not washed at once, but is only liberated as far as possible from the liquor by pressing or stretching, whereafter it is oiled on the grain with mineral oil alone, and on the inner side with mineral oil to 40 which sulfurized oils have been added, and the leather is then dried. When dry the leather can be impregnated with ceresin, paraffin or other mineral fats, for special purposes, and then washed with water.

45 If it is desired to reduce the reacting property of the ferric salts contained in the leather to such an extent that vegetable tanning, or similar substances, for example cellulose extracts or neradol can only exercise a weak action on said ferric salts, a sufficient quantity of a salt of alkaline reaction is added to the water used for the last 50 washing, and the leather is allowed to remain in this weak alkaline solution until on a fresh cut no, or but little, black coloring is produced with a neutral tanning substance. Thereafter the leather is treated according to the purpose for which it is to be used.

60 Owing to the close character of the grain caused by the tanning and finishing process it is possible to finish leather tanned with ferric salts on the inner or flesh side.

If the leather tanned with ferric oxid 65 salts is treated with reducing agents, for

instance with a 3% solution of sodium thiosulfate, if necessary after a preliminary treatment with a diluted acid solution for instance with a 5% solution of sulfuric acid, the ferric oxid salts in the outer layers will 70 be reduced into ferro-salts. In doing so the tanning salt is partly removed from the outer layers of the leather, and this exercises a bleaching action on the leather, producing, at the same time, a finer grain.

75 What I claim and desire to secure by Letters Patent of the United States is:—

1. The process for producing tough and durable leather from animal skins of all kinds which comprises treating the skins 80 with a solution of ferri-salts in the presence of an excess of chlorates such as sodium chlorate.

2. The process for producing tough and durable leather from animal skins of all 85 kinds which consists in preliminarily treating the depilated decalcified skins with weak salts of alkaline reaction and then tanning said skins in a solution of ferri-salt in the presence of an excess of some oxidizing 90 agent.

3. The process for producing tough and durable leather from animal skins of all kinds which consists in tanning the skins 95 with a solution of ferri-salts in the presence of an excess of some oxidizing agent, and in washing out the uncombined ferri-salts after said leather has been dried and treated with fat.

4. The process for producing tough and durable leather from animal skins of all 100 kinds which consists in tanning the skins with a solution of ferri-salts in the presence of an excess of some oxidizing agent, and in washing out the uncombined ferri-salts, and 105 in treating said skins with alkaline solutions after they have been dried and treated with fat.

5. The process for producing tough and durable leather from animal skins of all 110 kinds which consists in tanning said skins in a solution of ferri-salts in the presence of an excess of some oxidizing agent, and in then treating the surface of the leather with reducing agents.

6. The process for producing tough and durable leather from animal skins of all kinds which consists in tanning said skins in a solution of ferri-salts in the presence of an excess of some oxidizing agent, in treating the surface of said skins with dilute acid 120 solutions, and then with reducing agents.

In testimony whereof I have signed my name to this specification in the presence of two subscribing witnesses.

WILHELM MENSING.  
Witnesses:

MARTA PICKEL,  
CLARE SIMON.